

## UNITED STATES PATENT OFFICE

CAMILLE DREYFUS AND WILLIAM R. BLUME, OF NEW YORK, N. Y., ASSIGNEES TO  
CELANESE CORPORATION OF AMERICA, A CORPORATION OF DELAWARE

## ORNAMENTAL FABRIC AND METHOD OF MAKING THE SAME

No Drawing.

Application filed June 26, 1928. Serial No. 288,530.

This invention relates to the production of brocade or differential luster effects on fabrics of simple weave which fabric is made of yarns containing organic derivatives of cellulose, whereby lusters are produced on the fabric which are not appreciably affected by the ordinary laundering processes.

An object of our invention is to produce matte effects by the use of a water insoluble paste containing a mineral effect material.

A further object of our invention is to produce differential lusters without recourse to elaborate weaving processes, such as by means of Jacquard looms, on fabrics containing 15 yarns of organic derivatives of cellulose by the use of the matte printing paste. Other objects of our invention will appear from the following detailed description.

In accordance with our invention, we treat 20 a fabric containing organic derivatives of cellulose with a paste containing a mineral effect material and a water insoluble material that is dissolved in a solvent that does not have an appreciable solvent action on the organic derivative contained in the fabric, and preferably, but not necessarily, a plastifier or softening agent to impart suppleness to the film produced from the paste.

The fabric to be treated in accordance with 30 our invention may contain yarns of any suitable organic derivatives of cellulose such as cellulose esters and cellulose ethers. Examples of organic esters of cellulose are cellulose acetate, cellulose formate, cellulose pro- 35 pionate and cellulose butyrate. Examples of cellulose ethers are ethyl cellulose, methyl cellulose and benzyl cellulose. The fabric may consist of yarns made of one or more of these organic derivatives. The fabric may also be

40 a mixed fabric containing yarns of any of these organic derivatives of cellulose and yarns made of other fibres such as silk, cotton, wool or reconstituted cellulose (rayon). Examples of such fabrics are mixed cellulose 45 acetate and silk and mixed cellulose acetate and cotton.

Any suitable mineral effect material may be used in the matte printing paste. If color 50 is not desired to be imparted in the fabric, the paste may contain white pigments such

as zinc oxide or barium sulphate. If colors are desired, any suitable colored pigments such as is used in the paint art may be employed. The printing paste may also contain, if desired, dyes for the fabric to be 55 treated.

Any suitable water insoluble material may be used as thickener in the paste. While we have found cellulose nitrate to be preferred, other materials such as cellulose ethers may 60 be employed. However, it is important to use as the thickening material a substance which is soluble in some solvent that does not exert an appreciable solvent action on the organic derivative of cellulose contained in 65 the fabric.

The solvent for the water insoluble matter that may be used in preparing the paste should not exert an appreciable solvent action on the organic derivative contained in 70 the fabric. Thus if cellulose nitrate is used as an ingredient of the paste, a solvent consisting of alcohol and ether may be used. If cellulose ethers, such as ethyl cellulose are to be employed in the printing paste, benzene or 75 toluene may be used as the solvent. Obviously the paste containing cellulose ether and benzene or toluene will be used for printing a fabric that contains the organic esters of cellulose, but which does not contain the 80 cellulose ethers.

Of the plastifiers or softening agents that may be employed, the following may be mentioned: camphor, triphenyl phosphate, tri- 85 cresyl phosphate, dibutyl tartrate, diethyl phthalate, triacetin, etc. One or more of these plastifiers may be used. If desired medium and/or high boiling solvents may also be added.

The paste may be applied over the whole 90 surface of the fabric to be treated, in which case a fabric of uniformly dull luster will be obtained. If differential luster is desired, the matte printing paste will be applied locally by any suitable method such as by printing with engraved or embossed rolls, plates or blocks or by brushing or spraying through stencils having appropriate designs therein.

The paste may be applied to a fabric that has a normal luster with eminently satisfac-

tory results. However, for soft handle, the paste is preferably applied either locally or over the whole surface of a fabric, which has been previously delustered by any appropriate process, since delustered fabric has a softer handle than fabric of normal luster. As an example of a mode of delustering a fabric consisting of yarns of cellulose acetate, it is pointed out that the treatment of this material with wet steam or hot water at or near 100° C. will produce satisfactory delustered effects.

When the matte printing paste is applied locally over delustered fabric containing cellulose acetate, the unprinted portion of the fabric may be relustered by any suitable method. Since this application is not limited to the method of relustering such fabric, only a few methods of doing this will be described. The treatment of the fabric with dry steam above 100° C. will cause suitable relustering. In general the treatment of the fabric with substances that are capable of forming solutions with the organic derivative employed in the fabric will cause relustering of the same. Examples of such materials are aqueous solutions of formic acid, acetic acid, succinic acid, citric acid or sulpho cyanide such as sodium, ammonium or calcium sulpho cyanides. Likewise other organic substances such as aniline, phenol, aqueous acetone, etc. may be employed.

Where the matte paste has been applied to the fabric a dull matte effect is produced, which does not become relustered by the ordinary treatments to which fabrics are subjected, such as laundering, which includes both washing and ironing.

The fabric may be dyed prior to or after application of the paste, and the paste may contain differently colored pigments and/or dyes, whereby the designs that are produced are accentuated both by difference of luster and by difference of color. Merely by way of illustration and without limiting our invention thereto, the following specific example is given.

#### Example

A satin fabric made wholly of yarns of cellulose acetate and which has been previously dyed a golden maize color, is delustered by exposing the same to the action of wet steam somewhat below 100° C. The fabric is then locally printed with a matte printing paste consisting of cellulose nitrate, zinc oxide and a mixture of ethyl alcohol and ether to form a composition of the required consistency. For imparting suppleness to the printed portion, a suitable plastifier in amount equal to 10-60% of the weight of the cellulose nitrate may be added to the paste. After the paste on the fabric is dried, the printed fabric is padded or printed over its

entire surface with a relustering agency containing:

|                        | Parts |
|------------------------|-------|
| Calcium sulpho cyanide | 300   |
| Water                  | 100   |
| Gum arabic (1:1)       | 600   |

or else the relustering agency may be made up as follows:

|                               | Parts   |
|-------------------------------|---------|
| Acetic acid                   | 1 to 30 |
| Wheat starch thickening (15%) | 70      |
| Water                         | 0 to 20 |

After the application of the relustering agency, the fabric is dried and steamed. The part of the fabric that is printed with the matte paste is protected against relustering while the unprinted part becomes lustrous. There is thus produced a fabric having a dull figure against a golden lustrous background. If desired the background may be printed with the matte paste and designs left unprinted, whereby the reverse effect is obtained.

It is to be understood that the foregoing detailed description is given merely by way of illustration and that many variations may be made therein without departing from the spirit of this invention.

Having described our invention what we claim and desire to secure by Letters Patent is:

1. Method of producing matte effects upon fabrics containing organic derivatives of cellulose comprising delustering said fabric and then applying to said fabric a paste containing a water insoluble thickening agent, a pigment, and a solvent for said thickening agent which is a nonsolvent for the organic derivatives of cellulose contained in the fabric.

2. Method of producing matte effects upon fabrics containing cellulose acetate comprising delustering said fabric and then applying to said fabric a paste containing a water insoluble thickening agent, a pigment and a solvent for said thickening agent which is a nonsolvent for the cellulose acetate contained in the fabric.

3. Method of producing permanent matte effects upon fabrics containing cellulose acetate comprising delustering said fabric and then applying a paste containing cellulose nitrate, a softening agent, zinc oxide and a solvent for said cellulose nitrate which is a nonsolvent for the cellulose acetate contained in the fabric.

4. Method of producing brocade effects on fabrics containing cellulose acetate comprising delustering said fabric locally, applying a paste containing a water insoluble thickening agent, a pigment and a solvent for said thickening agent which is a nonsolvent for the cellulose acetate contained in the fabric and then subjecting the fabric to a relustering agency.

5. Method of producing brocade effects on  
fabrics containing cellulose acetate comprising  
delustering said fabric locally, applying  
a paste containing cellulose nitrate, a soft-  
tening agent, a pigment and a solvent for said  
cellulose nitrate which is a nonsolvent for  
the cellulose acetate contained in the fabric  
and then subjecting the fabric to a reluster-  
ing agency.

10 In testimony whereof, we have hereunto  
subscribed our names.

**CAMILLE DREYFUS.**  
**WILLIAM R. BLUME.**

15

20

25

30

35

40

45

50

55

60

65